

## UNITED STATES PATENT OFFICE

GRINNELL JONES, OF CAMBRIDGE, MASSACHUSETTS, ASSIGNOR TO PACIFIC MILLS, OF LAWRENCE, MASSACHUSETTS, A CORPORATION OF MASSACHUSETTS

## METHOD AND MATERIAL FOR PREVENTING THE TARNISHING OF SILVERWARE

No Drawing.

Application filed July 11, 1929. Serial No. 377,629.

Silverware will tarnish in a short time merely from exposure to ordinary atmosphere even if wrapped in bags and packed in closed drawers or trunks as usual. When stored for the summer or other extended period in safe deposit vaults, or elsewhere, silverware usually becomes coated with a tarnish so thick and adherent that cleaning is a long task. In the case of silverware elaborately embossed or engraved, complete cleaning is impossible by ordinary means without serious injury to the design, especially as the cleaning operation must be repeated at each tarnishing.

Many have attempted to devise means to prevent this tarnishing but none of the inventions heretofore patented or conceived has been sufficiently successful to come into general use. Much time and labor is constantly being expended in cleaning silverware on its withdrawal from storage or after it has lain idle.

It has long been known that silver tarnish consists in most cases of sulphide of silver and inventors have conceived the idea of preventing the tarnishing of silver and the wasteful cycle of polishing, storing and repolishing silver by preventing the formation of the tarnish.

The air and dust particles, especially in cities, contain minute traces of sulphur and sulphur compounds such as hydrogen sulphide or sulphur dioxide. Silver has such a very great chemical affinity for sulphur that it is capable of extracting these minute traces of sulphur from the air or from dust particles with the formation of silver sulphide and thereby becomes tarnished.

Some of the attempts to protect silver against tarnishing have been based on the idea of making a gas-tight container to prevent access of sulphur fumes to the silver. But such containers are cumbersome and awkward and permit access of sulphur fumes to the silver every time the container is opened to replace the silver articles so that they are only partially effective.

Another method which is in use is to cover the silverware with a transparent lacquer.

Although such lacquers are partially successful in preventing tarnish, they cannot be used on table ware because the lacquers will not stand the wear and washing to which they must be subjected.

It has also been suggested that the silverware should be wrapped in a bag impregnated with chemicals which dissolve or decompose silver sulphide so that the silverware when withdrawn will be free from tarnish. A bag impregnated with potassium ferrocyanide, potassium cyanide and glycerine has been suggested for this purpose. Potassium cyanide is an excellent solvent for silver sulphide and is, therefore, effective in detarnishing silver, but owing to the extremely poisonous nature of potassium cyanide, such a bag could not be used safely in the home and such a bag would soon lose any effectiveness it might have owing to the instability of potassium cyanide when exposed to air containing even traces of carbon dioxide. Another variation of this idea is to impregnate a paper with metallic zinc which in the presence of moisture and a soluble electrolyte is capable of decomposing silver sulphide.

Other attempts have been based on the idea that a cloth may be treated with a substance which will absorb and combine with the sulphur or sulphur compounds in the air and thus protect silverware enclosed within the treated cloth. Among the substances which have been suggested for this purpose are the oxide of lead, oxide of zinc, oxide of iron, borax, caustic alkalies, acetate of zinc, and chloride of zinc. I have found by repeated and careful experiments that although some of these substances will combine with and absorb sulphur compounds, the protection which they give is imperfect and temporary. I have also tried many other substances which, so far as I am aware, have never been used for this purpose and which are capable of forming insoluble sulphides, including cadmium, bismuth, copper and antimony in the form of metal, or oxides or salts and find that although a cloth impregnated with these substances will give some temporary protection to silverware enclosed

therein, the protection is imperfect and too short-lived to give satisfaction to the purchaser of such a cloth. The difficulty with all of these substances is that silver has a much greater chemical affinity for sulphur than any of the materials hitherto used to impregnate the cloth so that the sulphur will be passed on by the impregnating materials to the silverware in contact with the cloth, especially if the cloth is slightly moist.

I have found by extended experiments not only with the metals above described but with many other metals that this transfer takes place. The attraction of silver for sulphur exceeds that of all other usable metals so that silverware should tarnish in time from contact with the sulphide of any other usable metal. I have found, however, that if silver (or silver oxide or other salt of silver which will form silver sulphide, when exposed to the usual atmosphere or dust containing sulphur) is precipitated on or preferably throughout a bag or other wrapping and the bag or wrapping is placed around silverware that the silverware will not tarnish. I believe that the silver or silver salt in its finely divided state unites more readily with sulphur than does a solid block of silver, as a spoon, and that the finely divided silver, or silver compound, when once united with the sulphur will not pass the sulphur along to the silverware to be protected. Thus I have found sterling silver in bags in which silver or silver oxide has been precipitated will give protection for sixteen months and probably much more.

The above statement of the reasons for the success of my bags I believe to be true but whatever the cause, the fact is that bags impregnated according to my invention do give long protection which bags impregnated with other materials do not.

I deposit the silver or silver compound which acts as a sulphur absorbent on the cloth in finely divided but solid, insoluble, and adherent form which leaves the cloth in a soft and pliable condition and attractive in appearance and feel. I prefer to use a napped cotton cloth of close weave so that the interstices shall be a minimum, but fabrics of other materials or of other construction may be used, such as paper or felt.

To prepare a silver protecting cloth in accordance with my invention, I take a suitable napped cotton cloth and pass it through a solution containing twelve ounces of silver nitrate dissolved in a gallon of water and then pass the cloth through a squeeze roll or wringer to remove the excess of silver nitrate solution. Then without drying the cloth, I pass it into a hot alkaline solution of sodium carbonate containing 2% of sodium carbonate, thereby causing the silver to be precipitated on and in the cotton

fibers as a solid, insoluble, adherent compound of silver. Then the cloth is repeatedly washed with water to remove all excess of alkali and of other soluble substances. The cloth is then dried and is ready for use to wrap around silverware or as a lining for drawers, cupboards, or boxes, or if preferred, may be manufactured into bags with suitable draw strings or other well known devices to ensure tight closing of the bags.

It will, of course, be understood that the procedure given above is illustrative only and that the procedure may be varied without departing from the spirit of my invention. Thus, by using a weaker solution of silver nitrate the cost of the cloth will be reduced with some diminution of the length of time that the cloth will give perfect protection. Other soluble silver salts can be used instead of silver nitrate. The concentration of the sodium carbonate solution and the time and temperature of the treatment of the cloth with the sodium carbonate solution may be varied within wide limits. Other precipitating reagents may be used instead of sodium carbonate. Reducing agents which will change the silver compounds to metallic silver in whole or in part may be used if desired. Formaldehyde is suitable for this purpose although other reducing agents may be used if desired.

The term "impregnated" includes surface impregnation except where limited by the context.

Silver in any combination which will combine freely with sulphur as it occurs in the atmosphere or dust on exposure under ordinary conditions, is included in my invention as an impregnating material.

I have used the term "silver constituent" in the claims to include metallic silver or suitable compounds thereof and also mixtures of silver with suitable silver compounds. Some silver compounds would attack the hands of the user or poison the user or destroy the bags and would obviously be unsuitable to use unless changed by further chemical treatment.

In this specification I have described my preferred method of impregnation by precipitating a suitable compound practically insoluble in water in the fabric. This method I have found to have many advantages. A material impregnated with a compound insoluble in water in finely divided form may be washed without loss of material and presents a very large surface for contact with the tarnishing gases or dust while a fabric treated with a water soluble salt of silver without further treatment is almost certain to crystallize and when it unites with sulphur will usually produce an acid which is highly undesirable. Nevertheless, some protection is given even by im-

pregnated with suitable soluble salts of the tarnishing gases in the atmosphere in silver.

In view of the expense of the silver impregnated cloth, and the selling advantage of variety of color in the wrappers, it will often be desirable to make impregnated pockets fitted to hold one or more articles of silverware and wrap the pockets containing the silver in an unimpregnated wrapper.

10. If for any reason it is desired to produce a bag of a color which cannot be produced by a complete impregnation according to my invention, a surface impregnation on one side of the cloth only may be used and 15 will result in material protection.

I claim:

1. A fabric for protecting silverware from tarnish comprising a material suitable for wrapping, impregnated with a silver 20 constituent in a combination or condition which will combine with the tarnishing gases in the atmosphere accessible to the silverware wrapped therein.

2. A fabric for protecting silverware from 25 tarnish comprising a material suitable for wrapping, impregnated with a silver constituent insoluble in water in a combination or condition which will combine with the tarnishing gases in the atmosphere accessible to the silverware wrapped therein.

3. A fabric for protecting silverware from tarnish comprising a material suitable for wrapping, impregnated with an insoluble compound of silver in a combination or 30 condition which will combine with the tarnishing gases in the atmosphere accessible to the silverware wrapped therein.

4. A fabric for protecting silverware from tarnish comprising a material suitable for 40 wrapping, impregnated with oxide of silver.

5. A package for silverware having in combination an exterior casing and a series 45 of bags impregnated with a silver constituent in finely divided form which will combine with the tarnishing gases in the atmosphere in contact with them.

6. A package for silverware having in combination an exterior casing and a series 50 of bags impregnated with a silver constituent insoluble in water in finely divided form which will combine with the tarnishing gases in the atmosphere in contact with them.

7. A package for silverware having in 55 combination an exterior casing and a series of bags impregnated with an insoluble compound of silver in finely divided form which will combine with the tarnishing gases in the atmosphere in contact with them.

8. A package for silverware having in 60 combination an exterior casing and a series of bags impregnated with oxide of silver in 65 finely divided form which will combine with

the tarnishing gases in the atmosphere in contact with them.

9. A package for silverware comprising a material suitable and adapted for wrapping the silverware to be protected, impregnated with a silver constituent which will combine with the sulphur atoms in the atmosphere accessible to the silverware wrapped therein. 70

10. A package for silverware comprising a material suitable and adapted for wrapping the silverware to be protected, impregnated with a silver constituent insoluble in water which will combine with the sulphur atoms in the atmosphere accessible to the silverware wrapped therein. 75

11. A package for silverware comprising a material suitable and adapted for wrapping the silverware to be protected, impregnated with an insoluble compound of silver 80 which will combine with the sulphur atoms in the atmosphere accessible to the silverware wrapped therein. 85

12. A package for silverware comprising a material suitable and adapted for wrapping the silverware to be protected, impregnated with oxide of silver. 90

13. The method of protecting silverware from tarnish which consists in wrapping the silverware in a fabric impregnated with a silver constituent in a finely divided form 95 which will combine with the sulphur atoms in the atmosphere accessible to the silverware.

14. The method of protecting silverware from tarnish which consists in wrapping the silverware in a fabric impregnated with a silver constituent insoluble in water in a finely divided form which combine with the sulphur atoms in the atmosphere accessible to the silverware. 100

15. The method of protecting silverware from tarnish which consists in wrapping the silverware in a fabric impregnated with an insoluble compound of silver in a finely 110 divided form which will combine with the sulphur atoms in the atmosphere accessible to the silverware.

16. The method of protecting silverware from tarnish which consists in wrapping the silverware in a fabric impregnated with oxide of silver in a finely divided form. 115

17. The method of protecting silverware from tarnish which consists in wrapping the silverware in a fabric impregnated with 120 a substance containing silver atoms in a form which will combine with the tarnishing gases in the atmosphere accessible to the silverware and prevent them from combining with the silver on the surface of the 125 silverware.

GRINNELL JONES.